# EUROPEAN PATENT SPECIFICATION

(11) **EP 0 701 635 B1**
(45) Date of publication and mention of the grant of the patent: **06.05.1998**
(21) Application number: 94915259.9
(22) Date of filing: 01.06.1994
(51) Int. Cl.: C25C 3/12, C25C 3/08

(54) **TREATING PREBAKED CARBON ANODES FOR ALUMINIUM PRODUCTION**
BEHANDLUNG VON VORGEBRANNTEN ANODEN FÜR DIE HERSTELLUNG VON ALUMINIUM
TRAITEMENT D'ANODES DE CARBONE PRECUITES POUR LA PRODUCTION D'ALUMINIUM

(30) Priority: 02.06.1993 EP 93810401; 02.08.1993 EP 93810545; 28.03.1994 US 218679
(43) Date of publication of application: 20.03.1996
(73) Proprietor: MOLTECH Invent S.A., 2320 Luxembourg (LU)
(72) Inventor: MANGANIELLO, Fausto Alures, I-09010 Portoscuso (IT); DURUZ, Jean-Jacques, CH-1204 Geneva (CH); BELLO, Vittorio Alures, I-09010 Portoscuso (IT)
(74) Representative: Cronin, Brian Harold John
(86) International application number: IB9400134
(87) International publication number: WO9428200

(56) References cited:
- WO-A-93/25731
- DE-A- 2 042 810

## Description

### Field of the Invention

This invention relates to components, in particular prebaked carbon anodes and sidewalls, of electrolytic cells for the production of aluminium especially by the electrolysis of alumina in a molten fluoride electrolyte such as cryolite, and is particularly concerned with improving the resistance to oxidation of the sides and top of prebaked anodes and of sidewalls which are exposed to air and oxidising gases during cell operation.

### Background Art

Aluminium is produced conventionally by the Hall-Héroult process, by the electrolysis of alumina dissolved in cryolite-based molten electrolytes at temperatures up to around 950°C. In Hall-Héroult cells, the anodes are usually prebaked carbon blocks that are consumed by the electrochemical reaction, corroded by contact with the electrolyte and disintegrated by the evolved oxidising gases.

Prebaked anodes for aluminium production are made of a matrix of petroleum coke with pitch as binder. Their production involves various phases including preparing and treating the starting materials, mixing, forming and calcining at high temperature, followed by securing the current supply member by rodding.

The production of aluminium involves a complex reaction summarised by the relationship: ${\text{Al}}_{\text{2}} {\text{O}}_{\text{3}} {\text{+ C → Al + CO}}_{\text{2}}$ with a theoretical consumption of 0.334 kg of the anodic carbon per kilo of product aluminium. However, the real anode consumption is 40-50% greater, and amounts to about 20% of the production cost of the aluminium.

The above-stoichiometric consumption of carbon stems from a series of secondary reactions or parasitic phenomena, subdivided as follows:
- oxidising reactions with oxygen from the air which contacts the upper part of the anode and, if the latter is non-protected, reacts (C + O₂ → CO₂) ;
- carbo-oxidation reactions with CO₂ at the surface of the anode immersed in the electrolyte : the so-called "Boudouard equilibrium" (C + CO₂ → CO) ; and
- selective oxidation of pitch coke with respect to petroleum coke, with consequent release of carbon particles which tend to deposit on the surface of the electrolyte, interfering with the electrolysis and increasing the electrolyte temperature.

In view of the importance of the anode consumption on the economics of the Al-production process, great efforts have been made in recent years to study the problem. This has led to the anode consumption being correlated with a series of variables, including the electrolyte temperature, the permeability of the anode to air, and the thermal conductivity of the anode. It is now possible, based on equations, to make estimates of anode consumption which correspond approximately to the values found in industrial practice.

It is widely believed that the major component of the increased anode consumption is due to oxidation of the anode surface in contact with air. A typical distribution of the specific net consumption of carbon (with the best state-of-the-art protective aluminium coatings) is :

| Consumption | kgC/kg Al | % |
|---|---|---|
| Electrochemical | -0.334 | -76.0 |
| Current efficiency | -0.037 | -8.4 |
| Oxidation | -0.051 | -11.6 |
| Carbo-oxidation | -0.018 | -4.0 |
| Specific Net Consumption | | -0.440 |

Prebaked carbon anodes contain metallic impurities originating from the starting materials, which impurities undesirably influence the anode consumption. In particular, V, Fe, S and especially Na exert a catalytic activity influencing the anode oxidation reaction, favourising the attack by O₂.

Many attempts have been made to develop techniques to reduce the oxidation of prebaked carbon anodes in order to improve the efficiency, for instance by including additives in the coke-pitch mixture.

The addition of phosphorous, as phosphate or phosphoric acid, has a beneficial effect on anode consumption but undesirably pollutes the product aluminium and reduces current efficiency. For this reason, phosphorous-based treating agents such as that described in US Patent 4 439 491 have not been successful as oxygen inhibitors for prebaked carbon anodes used for aluminium production.

AlF₃ has been proposed as additive on account of the fact that it is non-polluting to the bath. A reduction of the carbon consumption is obtained, but is attributed to the fact that AlF₃ vapours reduce the differential reaction between coke and pitch, so the available saving is small because there is no reduction of the main oxidation.

Other compounds such as AlCl₃ in an amount of 1-3%, or SiO₂ as H₂SiO₃ in an amount of 0.2 to 1%, have also been tried, but without giving satisfactory results.

Boron, principally in the form of B₂O₃ and boric acid (H₃BO₃) has also been found to inhibit the catalytic agents present (such as NaO₂, FeO, and V₂O₅) by forming stable alloys therewith.

By including boron compounds in prebaked carbon anodes with a concentration which in some cases is 0.2 to 0.3 weight% or more of the entire anode, it has been possible to reduce the oxidation by up to about 50%. See for example US Patent 4 613 375, which proposed adding 0.5 to 1.5 weight% of inorganic additives including B and B₂O₃, and DE-A-35 38 294, which proposed doping the carbon making up the anode with manganese and boron or with cobalt and boron as corrosion inhibitors, with each element present in an amount of at least 0.1 and preferably at least 0.5 weight% of the carbon. These proposals however are still unsatisfactory because the maximum permissible boron content for an aluminium production anode should not exceed about 60ppm in the product aluminium, which corresponds to a maximum of about 150ppm in the entire anode.

For other applications, such as carbon anodes for arc furnaces, where boron pollution is not a problem, it has been proposed to improve the oxidation resistance by including boron in an amount of as much as about 3 weight% of the entire carbon body. See for example US Patent 4 770 825. Obviously, this is totally unacceptable for aluminium production anodes.

Protective coatings for aluminium production anodes have also been proposed, notably a fused layer of aluminium on the anode surfaces. This technique is economically questionable, as it requires from about 0.8 to 1.0 g Al/cm² of the anode surface, and the poor wettability of carbon by the fused aluminium leads to problems in the uniformity of such coatings. Nevertheless, coating with aluminium has been the most widely accepted expedient to date to reduce anode oxidation.

Another proposed protective coating consists of alumina, but this has the disadvantage of creating a thermal insulation around the anode, leading to local overheating and acceleration of the oxidation process.

Attempts to coat the anodes with B₂O₃-based protective coatings applied onto the carbon surfaces have not been successful. US Patent 3 852 107 describes spraying a coating 0.5 to 5mm thick onto a pre-heated anode, the spray mixture comprising a matrix of a boron compound and a refractory filler such as a carbide.

DE-A-2,042,810 discloses impregnating a carbon anode for aluminium production with boron compounds followed by heat treatment to form boron carbide within the pores. Impregnation took place for several hours with the solution near boiling point, providing impregnation to 8-10 cm followed by drying for several hours and preferably baking in an inert atmosphere at 900-1000°C for several hours.

To overcome the drawbacks of previous attempts to make use of boric acid or salts thereof, DE-A-28 09 295 described coating a carbon body such as a prebaked anode for aluminium-production, by using a solution of ammonium pentaborate or ammonium tetraborate to produce a glassy coating of anhydrous boric acid (B₂O₃). Such coatings initially reduce the reactivity of the anode surface with oxygen, but the effect is short-lived and, once the coating has been worn away, is lost.

Such coatings remain on an external surface of the anode and can easily be mechanically damaged during transport of the anode and its installation in the cell. Also, such coatings are not perfectly impervious to gas, and cannot protect the anode from oxidation.

Problems like those described above for prebaked carbon anodes apply also to the carbon cell sidewalls including a lower part submerged or the electrolyte and an upper part which is exposed to CO₂-enriched air, and which disintegrate and wear away as a result of attack by oxidising gases.

### Summary of the Invention

An object of the invention is to improve the resistance to oxidation of a preformed carbon anode or a cell sidewall for aluminium production by the incorporation of boron without the inherent drawbacks of the known proposals.

The invention provides a method of treating a cell component, in particular a prebaked carbon-based anode or sidewall, of an electrolytic cell for the production of aluminium, in particular by the electrolysis of alumina in a molten fluoride electrolyte such as cryolite, to improve the resistance thereof to deterioration during operation of the cell by the attack of air and oxidising gases released at the anode, using boron in acceptable amounts in the surface parts exposed in use to oxidising gases.

In the method according to the invention the surface of the component is contacted with a boron-containing solution which has a low surface tension providing an angle of contact of less than 90° with the carbon-based material to provide adequate wettability and facilitate penetration, said boron-containing solution being impregnated to a selected depth of 1 to 5 cm over the surface of the component to be protected, followed by drying.

The impregnation treatment of the invention provides a protected layer of one or several centimeters, wherein the boron penetrates in the pores into which oxidising air/gas enter.

The treatment applies in particular to prebaked carbon anodes which are liable to be subject to mechanical damage of the external layer during transport. With the treatment according to the invention, damage to the outer surface is not detrimental to the protection against oxidation, due to the thickness of the impregnation which provides a long-lasting protective effect as the anode wears away slowly during use.

The impregnation treatment applies also to the cell sidewalls, particularly the upper part of the cell sidewall that is exposed to air and the effect of oxidising gases during use, as well as the lower part exposed to carbo-oxidation reactions with CO₂ at the surface of the sidewall submerged in the electrolyte.

In the case of impregnating cell sidewalls, the protective effect can be enhanced by topcoating the impregnated sidewalls with a layer of refractory material e.g. particulate diboride in a colloidal carrier, such as titanium diboride in colloidal alumina, as described in WO 93/25731.

The boron-containing solution comprises a boron compound such as B₂O₃, boric acid or tetraboric acid dissolved in a solvent preferably selected from methanol, ethylene glycol, glycerin, water containing at least one surface-active agent, and mixtures thereof.

Good results have been achieved with boric acid and precursors of boric acid that form B₂O₃. Borates have not been found to give good results.

The solution preferably contains 5 - 60 weight% of the boron compound in particular using a solution at a temperature in the range from 10° to 120°C, preferably 20°C to 80°C, these conditions ensuring excellent penetration of the solution into the porous carbon. For solutions with 50-60 weight % of boron compounds, solvents like methanol, ethylene glycol or glycerin are used at a temperature of about 80°C or above.

It is advantageous to carry out the treatment with a heated solution in order to increase the solubility of the boron compound and decrease the treatment time. But this involves also heating the anode. Therefore, carrying the method out at ambient temperature is also convenient because no special heating equipment is required.

At low temperatures, solvents such as methanol, ethylene glycol and glycerin will be preferred, possibly with additives to enhance the solubility of the boron compound, and the treatment time may be extended to several hours. When water is used as solvent, surfactant agents in particular tensio-active cationic agents are used. Anionic tensio-active agents can also be used. Such agents should be devoid of components that would undesirably contaminate the aluminium produced and components that promote oxidation of the carbon. These surface-active agents may possibly be present together with other solubility improving agents such as tartaric acid or citric acid, and the solution may be heated to improve and to speed up the impregnation of the anode.

The use of surface active agents is an important factor to accelerate penetration of the solution and to obtain impregnation to a sufficient depth of several centimeters in only a few minutes, since long treatment times would make the process uneconomical.

The anode can be treated by immersion in the boron-containing solution for about 2 minutes to 1 hour for a heated solution, followed by drying. Usually, a single impregnation suffices, but the impregnation and drying may be repeated until the treated anode surface is saturated with the boron compound.

The treatment time depends principally on the exposed surface area of the anode and its porosity, as well as the temperature. It has been observed that prolonging the treatment does not significantly increase the boron concentration or the depth of penetration.

When a heated solution is used, it is advantageous to provide a thermostat-controlled heating installation for maintaining the solution at the desired temperature during the entire immersion time.

Anodes are conveniently impregnated simply by dipping them into the solution, which can take place in ambient conditions, but the impregnation may be assisted by the application of a pressure differential, by applying pressure or a vacuum. Other ways of speeding up impregnation can also be used, such as the application of ultrasounds.

In this way, the boron-containing solution impregnates the carbon anode to a depth of 1-5 cm, for example approximately 2 to 4 or 5cm, with a concentration of boron in the impregnated surface of the carbon anode in the range from 200ppm to 0.35%, or possibly even higher. Even with the highest achievable levels of boron concentration, the problem of process contamination is avoided because the protective boron compounds are present only in the top and side surfaces of the anode needing protection, and only to a depth of several centimeters.

By impregnating the parts of the anode to be protected - namely the side and top surfaces - with a small quantity of the boron compound to a depth of one or several centimeters, a long-lasting protective effect is achieved because the surfaces exposed to oxygen wear away very slowly over a long period, while avoiding undesirable contamination of the aluminium produced.

The anode is usually made of petroleum coke and pitch, the anode having an open porosity in the range 5% to 30%, preferably from 5 to 20%. The porous material making up the anode may also be a composite carbon-based material comprising at least one further component such as refractory oxycompounds, in particular alumina. Examples of such materials are described in WO 93/25494.

The impregnation treatment of a pre-baked anode according to the invention is made after calcinining where the anode surface has highest porosity, so improving the penetration of the solution to a depth of one or several centimeters.

Oxidation of the anodes increases with porosity. Thus, with the impregnation treatment, the most porous part of the anode which is most prone to damage by oxidation is protected. In other words, more porous parts of the surface to be protected are penetrated more and deeper by the boron-containing solution, providing greater protection where needed.

The intake of the boron-containing solution into the anode can monitored by checking the level of the solution, or simply by the time of immersion for a given solution and an anode of given porosity.

The top and side surfaces of the anode can be immersed in the boron-containing solution simply by dipping the anode upside down in the solution. There is no need to treat the bottom of the anode where the electrochemical reaction takes place. In this way, only those parts of the anode which need protection are treated in a simple way, and the amount of boron in the anode (and hence in the aluminium produced) is minimized.

The invention also concerns a prebaked carbon-based anode of an electrolytic cell for the production of aluminium, in particular by the electrolysis of alumina in a molten fluoride electrolyte such as cryolite, wherein the top and side surfaces of the anode are impregnated to a depth of 1 to 5cm, preferably about 2 to 4cm, with a boron compound, to improve the resistance thereof to consumption during operation of the cell by air and oxidising gases released at the anode. The central part and the lower surface of the anode are essentially devoid of the boron-containing compound.

Such an anode may be produced by the methods set out above, and may incorporate all of the features described in connection with the method.

The invention also concerns an electrolytic cell for the production of aluminium, in particular by the electrolysis of alumina in a molten fluoride electrolyte such as cryolite, comprising an anode or sidewall as set out above, the anode or sidewall being installed with the treated boron-containing surfaces of the anode in contact with air and oxidising gases released during operation of the cell.

### Detailed Description

To achieve an optimum protective effect against oxidation, several parameters of the treatment solution need to be balanced.

The concentration of the boron compound, in particular H₃BO₃ or B₂O₃, is important : greater concentrations provide a greater concentration gradient, favourising the kinetics of penetration of the solution into the porous anode. Solubility of the boron compounds can be increased by maintaining the solution at a suitable high temperature.

The coefficient of diffusion of the solution into the porous carbon structure and the wettability of the carbon by the solution will influence the rate and the degree of penetration. Solutions with low surface tension providing an angle of contact with the carbon of less than 90° provide adequate wettability and facilitate penetration. A suitable high solution temperature will also enhance diffusion of the solution.

Solvents with a low degree of inflammability are desirable. Should flammable solvents impregnate the carbon, this could lead to unwanted heat generation favorising oxidation of the carbon.

The type of solvent chosen directly influences the variability of the process parameters and in particular the results, especially the depth of penetration of the solution.

By using solvents selected from methanol, ethylene glycol, glycerin and mixtures thereof, at a temperature from 80° to 120°C, a concentration of 50-60 weight% of H₃BO₃ or B₂O₃ can be achieved in the solution, or about 20% when water with a surface-active agent is used as solvent. Such solutions have desirable physio-chemical properties, providing excellent impregnation by immersion of an anode in about 2-60 minutes. In these conditions, treatment of an anode having a porosity of about 15-18% and a surface area of 2-3m² produces an impregnation to a depth of about 3-4 cm with a boron concentration of several hundreds of ppm.

When water is chosen as solvent, a surfactant such as those available under the tradenames NONIDET P 40 and SPAN 85, from Fluka, and GLUCOPON 225, DEHYPON LS, QUAFIN LDM and QUAFIN CT, from Henkel, are used in order to achieve an acceptable low treatment time.

In practice, the treatment solution can first be prepared using metering means to mix the H₃BO₃ or B₂O₃ in the chosen solvent, in the desired proportions, in a container provided with a thermostatically-controlled heater and a mechanical mixer. The solution can then be heated to its use temperature in the range of 80° to 120°C, for example, and the hot solution transferred to a thermostatic vessel equipped with a level indicator.

Generally, a boron salt is added to the solvent in a quantity sufficient to guarantee saturation of the solution upon heating, leaving a deposit of the undissolved salt in the bottom of the vessel.

The anode to be treated is then dipped in the vessel, upside down, so its top and side surfaces are immersed in the hot solution. Immersion is continued for a set time, e.g. from 2-60 minutes, or until the level indicator has indicated a desired intake of the solution into the treated surfaces. The treated anode is then removed and dried. The vessel is then topped up to its initial level with hot solution from the container, ready for the treatment of another anode.

The vapors produced in the described conditions are non toxic and can be freely released into the air without a need for costly treatment installations.

The carbon consumption due to air-oxidation of anodes treated this way corresponds to about 12-15% with respect to the net consumption, which is comparable to what can be achieved with traditional aluminium protective coatings. Thus, the invention provides an excellent and long-lasting protective effect at much less cost and with less risk of imperfections in the protection than with aluminium coatings.

The components of the treatment solution are inexpensive and are non-polluting both for the aluminium production process and for the environment. The method is simple to carry out, and the treated surfaces are uniformly impregnated with the boron compounds, leading to reliability in use because of uniform wear to the exposed surfaces of the anode or sidewall. Also, as boron acts as a "negative catalyst", it is possible to make the anode and sidewall from carbon powder containing a higher content of vanadium, thereby reducing the cost of raw materials.

## Claims

1. A method of treating a carbon-based cell component of an electrolytic cell for the production of aluminium, in particular by the electrolysis of alumina in a molten fluoride electrolyte, to improve the resistance thereof to deterioration during operation of the cell by the attack of air and anodically-released oxidising gases, wherein the surface of the component is contacted with a boron-containing solution which has a low surface tension providing an angle of contact of less than 90° with the carbon-based material to provide adequate wettability and facilitate penetration, said boron-containing solution being impregnated to a selected depth of 1 to 5 cm over the surface of the component to be protected, followed by drying.

2. The method of claim 1, wherein the cell component is a prebaked carbon anode.

3. The method of claim 1, wherein the cell component is a sidewall.

4. The method of claim 1, wherein the boron-containing solution comprises a boron compound dissolved in a solvent selected from methanol, ethylene glycol, glycerin, water containing at least one surface-active agent, and mixtures thereof.

5. The method of claim 1, wherein the solution contains B₂O₃, boric acid or tetraboric acid.

6. The method of claim 1, wherein the solution contains 5 - 60 weight% of boron compound.

7. The method of claim 2, wherein the treatment is carried out by immersion of the anode in the boron-containing solution at a temperature in the range 10° to 120°C.

8. The method of claim 7, wherein the treatment is carried out by immersion of the anode in the boron-containing solution at a temperature in the range 20° to 80°C.

9. The method of claim 8, wherein the anode is immersed in the boron-containing solution for about 2 minutes to 1 hour.

10. The method of claim 8, wherein the intake of the boron-containing solution into the anode is monitored by checking the level of the solution.

11. The method of claim 8, wherein top and side surfaces of the anode are immersed in the boron-containing solution by dipping the anode upside down in the solution.

12. The method of claim 1, wherein the boron-containing solution impregnates the carbon component to a depth of approximately 2 to 4 cm.

13. The method of claim 1, wherein the concentration of boron in the surface of the carbon component is in the range from 200ppm to 0.35%.

14. The method of claim 2, wherein the anode is made of petroleum coke and pitch, or is a composite material comprising predominantly petroleum coke and pitch, the anode having an open porosity in the range 5% to 30%.

15. The method of claim 3, which comprises applying a coating of refractory boride on top of the surface of the sidewall impregnated with the boron-containing solution.

16. The method of claim 15, wherein a coating of particulate titanium diboride in colloidal alumina is applied to said surface.

17. A prebaked carbon-based anode of an electrolytic cell for the production of aluminium, in particular by the electrolysis of alumina in a molten fluoride electrolyte, wherein the anode has top and side surfaces which in use are exposed to oxidising gases, said top and side surfaces being impregnated to a depth of 1 to 5 cm with a boron compound to improve the resistance thereof to erosion during operation of the cell by air and anodically-released oxidising gases, wherein the concentration of boron in the impregnated surface is in the range from 200ppm to 0.35%, the anode having a central part and a lower surface part which are essentially devoid of the boron-containing compound.

18. The anode of claim 17, wherein the boron-containing compound is derived from B₂O₃, boric acid, and tetraboric acid.

19. The anode of claim 17, wherein the boron-containing compound impregnates the carbon anode to a depth of approximately 2 to 4 cm.

20. The anode of claim 17, 18 or 19, which is made of petroleum coke and pitch, or is a composite material comprising predominantly petroleum coke and pitch, the anode having an open porosity in the range 5% to 30%.

21. An electrolytic cell for the production of aluminium by the electrolysis of alumina in a molten fluoride electrolyte, comprising a component treated by the method of claim 1, which component's surface is impregnated to a depth of 1 to 5 cm, wherein the concentration of boron in the impregnated surface is in the range from 200ppm to 0.35%, the component being installed with its treated surface in contact with air and oxidising gases released during operation of the cell.

22. The cell of claim 21, wherein the component is a prebaked carbon anode.

23. The cell of claim 21, wherein the component is a sidewall.

24. The cell of claim 23, wherein the treated surface of the sidewall is coated with a coating of refractory boride.

25. The cell of claim 24, wherein the treated surface of the sidewall is coated with titanium diboride in dried colloidal alumina.

## Patentansprüche

1. Verfahren zur Behandlung einer auf Kohlenstoff basierenden Zellkomponente einer elektrolytischen Zelle zur Herstellung von Aluminium, insbesondere durch Elektrolyse von Aluminiumoxid in einem geschmolzenen Fluoridelektrolyten, um deren Widerstandsfähigkeit gegen das Verschlechtern während des Betriebs der Zelle durch den Angriff von Luft oder anodisch freigesetzten oxidierenden Gasen zu verbessern, bei dem die Oberfläche der Komponente mit einer borhaltigen Lösung in Kontakt gebracht wird, welche eine niedrige Oberflächenspannung aufweist, die einen Kontaktwinkel von weniger als 90° mit dem auf Kohlenstoff basierenden Material ergibt, um eine angemessene Benetzbarkeit zu gewährleisten und die Penetration zu erleichtern, wobei die Oberfläche der zu schützenden Komponente mit der borhaltigen Lösung bis zu einer ausgewählten Tiefe von 1 bis 5 cm imprägniert und anschließend getrocknet wird.

2. Verfahren gemäß Anspruch 1, bei dem die Zellkomponente eine vorgebrannte Kohlenstoffanode ist.

3. Verfahren gemäß Anspruch 1, bei dem die Zellkomponente eine Seitenwand ist.

4. Verfahren gemäß Anspruch 1, bei dem die borhaltige Lösung eine Borkomponente enthält, die in einem Lösungsmittel gelöst ist, das unter Methanol, Ethylenglykol, Glycerin, Wasser, das mindestens einen oberflächenaktiven Stoff enthält, und Mischungen daraus ausgewählt ist.

5. Verfahren gemäß Anspruch 1, bei dem die Lösung B₂O₃, Borsäure oder Tetraborsäure enthält.

6. Verfahren gemäß Anspruch 1, bei dem die Lösung 5 bis 60 Gew.-% der Borverbindung enthält.

7. Verfahren gemäß Anspruch 2, bei dem die Behandlung durch Eintauchen der Anode in die borhaltige Lösung bei einer Temperatur im Bereich von 10 bis 120 °C durchgeführt wird.

8. Verfahren gemäß Anspruch 7, bei dem die Behandlung durch Eintauchen der Anode in die borhaltige Lösung bei einer Temperatur im Bereich von 20 bis 80 °C durchgeführt wird.

9. Verfahren gemäß Anspruch 8, bei dem die Anode für etwa 2 Minuten bis zu 1 Stunde in die borhaltige Lösung eingetaucht wird.

10. Verfahren gemäß Anspruch 8, bei dem die Aufnahme der borhaltigen Lösung in die Anode durch das Überprüfen der Füllhöhe der Lösung überwacht wird.

11. Verfahren gemäß Anspruch 8, bei dem die Ober- und Seitenflächen der Anoden in die borhaltige Lösung eingetaucht werden, indem die Anode mit der Oberseite voran in die Lösung getaucht wird.

12. Verfahren gemäß Anspruch 1, bei dem die borhaltige Lösung die Kohlenstoffkomponente bis zu einer Tiefe von ungefähr 2 bis 4 cm imprägniert.

13. Verfahren gemäß Anspruch 1, bei dem die Konzentration des Bors in der Oberfläche der Kohlenstoffkomponente im Bereich von 200 ppm bis 0,35 % liegt.

14. Verfahren gemäß Anspruch 2, bei dem die Anode aus Petroleumkoks und Pech hergestellt ist, oder ein Verbundmaterial ist, das überwiegend Petroleumkoks und Pech enthält, wobei die Anode eine offene Porosität im Bereich von 5 % bis 30 % aufweist.

15. Verfahren gemäß Anspruch 3, welches das Aufbringen einer Beschichtung von hitzebeständigem Borid auf die Oberseite der Oberfläche der mit der borhaltigen Lösung imprägnierten Seitenwand umfaßt.

16. Verfahren gemäß Anspruch 15, bei dem eine Beschichtung aus partikulärem Titandiborid in kolloidalem Aluminiumoxid auf die Fläche aufgebracht wird.

17. Vorgebrannte auf Kohlenstoff basierende Anode einer elektrolytischen Zelle zur Herstellung von Aluminium, insbesondere durch Elektrolyse von Aluminiumoxid in einem geschmolzenen Fluoridelektrolyten, wobei die Anode Ober- und Seitenflächen aufweist, welche während des Gebrauchs oxidierenden Gasen ausgesetzt sind, wobei die Ober- und Seitenflächen bis zu einer Tiefe von 1 bis 5 cm mit einer Borverbindung imprägniert sind, um deren Widerstandsfähigkeit gegen Erosion während des Betriebs der Zelle durch Luft und anodisch freigesetzte oxidierende Gase zu verbessern, wobei die Konzentration des Bors in der imprägnierten Fläche im Bereich von 200 ppm bis 0,35 % liegt, wobei die Anode einen zentralen Teil und einen unteren Oberflächenteil aufweist, welche im wesentlichen frei von der borhaltigen Verbindung sind.

18. Anode gemäß Anspruch 17, bei der die borhaltige Verbindung von B₂O₃, Borsäure und Tetraborsäure abgeleitet ist.

19. Anode gemäß Anspruch 17, bei der die borhaltige Verbindung die Kohlenstoffanode bis zu einer Tiefe von etwa 2 bis 4 cm imprägniert.

20. Anode gemäß Anspruch 17, 18 oder 19, welche aus Petroleumkoks und Pech hergestellt ist, oder ein Verbundmaterial ist, das überwiegend Petroleumkoks und Pech enthält, wobei die Anode eine offene Porosität im Bereich von 5 % bis 30 % aufweist.

21. Elektrolytische Zelle zur Herstellung von Aluminium durch Elektrolyse von Aluminiumoxid in einem geschmolzenen Fluoridelektrolyten, enthaltend eine gemäß dem Verfahren von Anspruch 1 behandelte Komponente, wobei die Oberfläche der Komponente bis zu einer Tiefe von 1 bis 5 cm imprägniert ist, wobei die Konzentration des Bors in der imprägnierten Fläche im Bereich von 200 ppm bis 0,35 % liegt, und wobei die Komponente so installiert ist, daß sie mit ihren behandelten Flächen in Kontakt mit Luft und oxidierenden Gasen steht, die während der Operation der Zelle freigesetzt werden.

22. Zelle gemäß Anspruch 21, bei der die Komponente eine vorgebrannte Kohlenstoffanode ist.

23. Zelle gemäß Anspruch 21, bei der die Komponente eine Seitenwand ist.

24. Zelle gemäß Anspruch 23, bei der die behandelte Fläche der Seitenwand mit einer Beschichtung von hitzebeständigem Borid beschichtet ist.

25. Zelle gemäß Anspruch 24, bei der die behandelte Oberfläche der Seitenwand mit Titandiborid in getrocknetem, kolloidalem Aluminiumoxid beschichtet ist.

## Revendications

1. Une méthode de traitement d'un composant de cellule à base de carbone d'une cellule électrolytique pour la production d'aluminium, en particulier pour l'électrolyse d'alumine dans un électrolyte de fluorure fondu, pour en améliorer la résistance à la détérioration pendant le fonctionnement de la cellule par l'attaque de l'air et des gaz oxydants dégagés anodiquement, dans laquelle la surface du composant est mis en contact avec une solution contenant du bore qui possède une faible tension superficielle offrant un angle de contact inférieur à 90° avec le matériau à base de carbone pour donner une mouillabilité adéquate et faciliter a pénétration, ladite solution contenant du bore étant imprégnée jusqu'à une profondeur sélectionnée de 1 à 5 cm sur la surface du composant à protéger, suivi d'un séchage.

2. La méthode de la revendication 1, dans laquelle le composant de la cellule est une anode de carbone précuite.

3. La méthode de la revendication 1, dans laquelle le composant de la cellule est une paroi latérale.

4. La méthode de la revendication 1, dans laquelle la solution contenant du bore comprend un composé de bore dissout dans un solvant sélectionné parmi le méthanol, l'éthylène-glycol, la glycérine, l'eau contenant au moins un agent tensioactif, et leurs mélanges.

5. La méthode de la revendication 1, dans laquelle la solution contient du B₂O₃, de l'acide borique ou de l'acide tétraborique.

6. La méthode de la revendication 1, dans laquelle la solution contient de 5 - 60 % en poids de composé de bore.

7. La méthode de la revendication 2, dans laquelle le traitement est mené par immersion de l'anode dans la solution contenant du bore à une température dans l'intervalle de 10° à 120°C.

8. La méthode de la revendication 7, dans laquelle le traitement est mené par immersion de l'anode dans la solution contenant du bore à une température dans l'intervalle de 20° à 80°C.

9. La méthode de la revendication 8, dans laquelle l'anode est immergée dans une solution contenant du bore pendant environ de 2 minutes à 1 heure.

10. La méthode de la revendication 8, dans laquelle l'arrivée de solution contenant du bore dans l'anode est mesurée en vérifiant le niveau de la solution.

11. La méthode de la revendication 8, dans laquelle les surfaces supérieures et latérales de l'anode sont immergées dans la solution contenant du bore en trempant l'anode à l'envers dans la solution.

12. La méthode de la revendication 1, dans laquelle la solution contenant du bore imprègne le composant en carbone jusqu'à une profondeur d'approximativement 2 à 4 cm.

13. La méthode de la revendication 1, dans laquelle la concentration de bore à la surface du composant en carbone est dans l'intervalle de 220 ppm à 0,35%.

14. La méthode de la revendication 2, dans laquelle l'anode est réalisée en coke de pétrole et en brai, ou est un matériau composite comprenant de façon prédominante du coke de pétrole et du brai, l'anode possédant une porosité ouverte dans l'intervalle de 5% à 30%.

15. La méthode de la revendication 3, qui comprend l'application d'un revêtement en borure réfractaire sur le dessus de la surface de la paroi latérale imprégnée avec la solution contenant du bore.

16. La méthode de la revendication 15, dans laquelle un revêtement en diborure de titane particulaire dans de l'alumine colloïdale est appliqué sur ladite surface.

17. Une anode précuite à base de carbone d'une cellule électrolytique pour la production d'aluminium, en particulier pour l'électrolyse d'alumine dans un électrolyte de fluorure fondu, dans laquelle l'anode possède des surfaces supérieures et latérales qui pendant l'utilisation sont exposées aux gaz oxydants, lesdites surfaces supérieures et latérales étant imprégnées jusqu'à une profondeur de 1 à 5 cm avec un composé de bore pour en améliorer la résistance à l'érosion pendant le fonctionnement de la cellule par l'air et les gaz oxydants dégagés anodiquement, dans laquelle la concentration de bore à la surface du composant en carbone est dans l'intervalle de 220 ppm à 0,35%, l'anode possédant une partie centrale et une surface inférieure qui sont essentiellement dénuées de composé contenant du bore.

18. L'anode de la revendication 17, dans laquelle la solution contient du B₂O₃, de l'acide borique ou de l'acide tétraborique.

19. L'anode de la revendication 17, dans laquelle la solution contenant du bore imprègne le composant en carbone jusqu'à une profondeur d'approximativement 2 à 4 cm.

20. L'anode de la revendication 17, 18 ou 19, qui est réalisée en coke de pétrole et en brai, ou est un matériau composite comprenant de façon prédominante du coke de pétrole et du brai, l'anode possédant une porosité ouverte dans l'intervalle de 5% à 30%.

21. Une cellule électrolytique pour la production d'aluminium par l'électrolyse d'alumine dans un électrolyte de fluorure fondu, comprenant un composant traité par la méthode de la revendication 1, laquelle surface du composant est imprégnée jusqu'à une profondeur de 1 à 5 cm, dans laquelle la concentration de bore dans la surface imprégnée est dans l'intervalle de 220 ppm à 0,35%, le composant étant installé avec sa surface traitée en contact avec l'air et les gaz oxydants dégagés pendant le fonctionnement de la cellule.

22. La cellule de la revendication 21, dans laquelle le composant est une anode de carbone précuite.

23. La cellule de la revendication 21, dans laquelle le composant est une paroi latérale.

24. La cellule de la revendication 23, dans laquelle la surface traitée de la paroi latérale est revêtue avec un revêtement en borure réfractaire.

25. La cellule de la revendication 25, dans laquelle la surface traitée de la paroi latérale est revêtue avec du diborure de titane particulaire dans de l'alumine colloïdale séchée.
